



US009991041B2

(12) **United States Patent**  
**Hsieh et al.**

(10) **Patent No.:** **US 9,991,041 B2**  
(45) **Date of Patent:** **\*Jun. 5, 2018**

(54) **VARIABLE COUPLED INDUCTOR**

(71) **Applicant:** **CYNTEC CO., LTD.**, Hsinchu (TW)

(72) **Inventors:** **Lan-Chin Hsieh**, Kaohsiung (TW); **Cheng-Chang Lee**, Yunlin County (TW); **Chih-Hung Chang**, Miaoli County (TW); **Chih-Siang Chuang**, Hsinchu (TW); **Tsung-Chan Wu**, Hsinchu County (TW); **Roger Hsieh**, Hsinchu County (TW)

(73) **Assignee:** **CYNTEC CO., LTD.**, Hsinchu (TW)

(\*) **Notice:** Subject to any disclaimer, the term of this patent is extended or adjusted under 35 U.S.C. 154(b) by 0 days. days.

This patent is subject to a terminal disclaimer.

(21) **Appl. No.:** **14/967,307**

(22) **Filed:** **Dec. 13, 2015**

(65) **Prior Publication Data**

US 2016/0099099 A1 Apr. 7, 2016

**Related U.S. Application Data**

(63) Continuation of application No. 13/969,486, filed on Aug. 16, 2013, now Pat. No. 9,251,944.

(30) **Foreign Application Priority Data**

Aug. 21, 2012 (TW) ..... 101130231 A

(51) **Int. Cl.**

**H01F 27/24** (2006.01)  
**H01F 17/06** (2006.01)

(Continued)

(52) **U.S. Cl.**

CPC ..... **H01F 27/24** (2013.01); **H01F 3/14** (2013.01); **H01F 17/04** (2013.01); (Continued)

(58) **Field of Classification Search**

CPC ..... H01F 17/04; H01F 3/14; H01F 27/2823; H01F 27/24; H01F 38/023; H01F 2003/106 (Continued)

(56) **References Cited**

**U.S. PATENT DOCUMENTS**

6,510,109 B2 \* 1/2003 Ohmori ..... G11B 11/10534 360/234.7  
9,251,944 B2 \* 2/2016 Hsieh ..... H01F 17/04 (Continued)

*Primary Examiner* — Mangtin Lian

(74) **Attorney, Agent, or Firm:** Ming-Lee Teng; Litron Patent & Trademark Office

(57) **ABSTRACT**

A variable coupled inductor includes a first core, two conducting wires, a second core and a magnetic structure. The first core includes two first protruding portions, a second protruding portion and two grooves, wherein the second protruding portion is located between the two first protruding portions and each of the grooves is located between one of the first protruding portions and the second protruding portion. Each of the conducting wires is disposed in one of the grooves. The second core is disposed on the first core. A first gap is formed between each of the first protruding portions and the second core and a second gap is formed between the second protruding portion and the second core. The magnetic structure is disposed between the second protruding portion and the second core and distributed symmetrically with respect to a centerline of the second protruding portion.

**18 Claims, 9 Drawing Sheets**



- (51) **Int. Cl.**
- H01F 17/04* (2006.01)  
*H01F 3/14* (2006.01)  
*H01F 38/02* (2006.01)  
*H01F 27/28* (2006.01)  
*H01F 3/10* (2006.01)
- (52) **U.S. Cl.**
- CPC ..... *H01F 27/2823* (2013.01); *H01F 38/023* (2013.01); *H01F 2003/106* (2013.01)
- (58) **Field of Classification Search**
- USPC ..... 336/212, 178, 221  
See application file for complete search history.

(56) **References Cited**

U.S. PATENT DOCUMENTS

|              |     |         |              |       |             |  |
|--------------|-----|---------|--------------|-------|-------------|--|
| 2004/0085174 | A1* | 5/2004  | Decristofaro | ..... | H01F 3/14   |  |
|              |     |         |              |       | 336/178     |  |
| 2005/0151614 | A1* | 7/2005  | Dadafshar    | ..... | H01F 27/255 |  |
|              |     |         |              |       | 336/223     |  |
| 2005/0258927 | A1* | 11/2005 | Lu           | ..... | H01F 27/385 |  |
|              |     |         |              |       | 336/234     |  |

\* cited by examiner



Fig. 1



Fig. 2



Fig. 3



Fig. 4A



**Fig. 4B**



Fig. 5



**Fig. 6**



Fig. 7



Fig. 8

## 1

## VARIABLE COUPLED INDUCTOR

## CROSS REFERENCE TO RELATED APPLICATIONS

This application is a continuation of U.S. application Ser. No. 13/969,486, filed on Aug. 16, 2013, which claims the benefit of priority of Taiwan Application No. 101130231, filed Aug. 21, 2012, each of which is incorporated by reference herein in their entirety.

## BACKGROUND OF THE INVENTION

## I. Field of the Invention

The present invention relates to a variable coupled inductor and, in particular, to a variable coupled inductor can improve efficiency in both light-load and heavy-load situations.

## II. Description of the Prior Art

A coupled inductor has been developed for a period of time; however, it is not often used in the circuit board. As a more powerful microprocessor needs a high current in a small circuit board, a variable coupled inductor has been gradually used in the circuit board. A variable coupled inductor can be used to reduce the total space of the circuit board consumed by traditional coupled inductors. Currently, a coupled inductor can reduce the ripple current apparently, wherein a smaller capacitor can be used to save the space of the circuit board. As the DC resistance (direct current resistance, DCR) of the coupled inductor is low, efficiency is better in a heavy-load situation. However, as the flux generated by each of the dual conducting wires will be cancelled each other when the dual conducting wires are coupled, the inductance becomes low and the efficiency becomes worse in a light-load situation.

## SUMMARY OF THE INVENTION

One objective of present invention is to provide a variable coupled inductor that can increase the efficiency in both heavy-load and light-load situations to solve the above-mentioned problem.

In one embodiment, a variable coupled inductor is provided, wherein variable coupled inductor comprises a first core comprising a first protrusion, a second protrusion, a third protrusion, a first conducting-wire groove and a second conducting-wire groove, wherein the second protrusion is disposed between the first protrusion and the third protrusion, the first conducting-wire groove is located between the first protrusion and the second protrusion, and the second conducting-wire groove is located between the second protrusion and the third protrusion; a first conducting wire disposed in the first conducting-wire groove; a second conducting wire disposed in the second conducting-wire groove; a second core disposed over the first core, wherein a first gap is formed between the first protrusion and the second core, a second gap is formed between the second protrusion and the second core and a third gap is formed between the third protrusion and the second core; and a magnetic structure disposed between the second protrusion and the second core, wherein the magnetic structure is symmetric with respect to the central line of the second protrusion.

## 2

The present invention proposes that the magnetic structure is disposed between the second projection in the middle of the first core and the second core, wherein the magnetic structure is symmetric with respect to the central line CL of the second protrusion 102. Therefore, the initial-inductance of the variable coupled inductor can be enhanced and light-load efficiency can be improved by means of the magnetic structure.

In one embodiment, the material of the variable coupled inductor of the present invention can be a ferrite material to achieve a high-saturation current, and copper sheet is used as an electrode to reduce the DC resistance, so that the efficiency in heavy-load is improved.

## 15 BRIEF DESCRIPTION OF THE DRAWINGS

The foregoing aspects and many of the accompanying advantages of this invention will become more readily appreciated as the same becomes better understood by 20 reference to the following detailed description when taken in conjunction with the accompanying drawings, wherein:

FIG. 1 illustrates a variable coupled inductor in three dimensions in accordance with one embodiment of present invention;

FIG. 2 illustrates the variable coupled inductor in FIG. 1 where the second core is removed;

FIG. 3 illustrates the first core and the magnetic structure of the variable coupled inductor in FIG. 2;

FIG. 4A and FIG. 4B each illustrates a side view of the 30 variable coupled inductor in FIG. 1 where the second conducting wire is removed, wherein FIG. 4B shows a non-magnetic material is filled into the gaps between the second core and the first core;

FIG. 5 illustrates the relationships between the measured 35 inductances and the currents in the variable coupled inductor in FIG. 1;

FIG. 6 illustrates a three dimensional view of the first core and the magnetic structure in accordance with one embodiment of present invention;

FIG. 7 illustrates a three dimensional view of the first core and the magnetic structure in accordance with another embodiment of present invention; and

FIG. 8 illustrates a three dimensional view of the first core and the magnetic structure in accordance with yet another embodiment of present invention.

## DETAILED DESCRIPTION OF THE INVENTION

50 Please refer to FIG. 1 to FIG. 4A. FIG. 1 is a three dimensional view of a variable coupled inductor 1 according to one embodiment of the present invention. FIG. 2 is a three dimensional view of a variable coupled inductor 1 where the second core 14 is removed in FIG. 1. FIG. 3 is a three 55 dimensional view of a first core 10 and a magnetic structure 16 in FIG. 2. FIG. 4A is a lateral view of a variable coupled inductor 1 wherein two conducting wires 12 are removed in FIG. 1. As illustrated in FIG. 1 to FIG. 4A, the variable coupled inductor 1 comprises a first core 10, two conducting 60 wires 12, a second core 14 and a magnetic structure 16. The first core 10 comprises two first protrusions 100, a second protrusion 102 and two conducting-wire grooves 104, wherein the second protrusion 102 is located between the two first protrusions 100, and each of the two conducting-wire groove 104 is located between corresponding one of the two first protrusions 100 and the second protrusion 102, respectively. In other words, the second protrusion 102 is 65

located in the middle portion of the first core **10**. Each of the two conducting wire **12** is disposed in one of the two conducting-wire grooves **104**, respectively. The second core **14** is disposed over the first core **10** so that a first gap **G1** is formed between each first protrusion **100** and the second core **14** and a second gap **G2** is formed between the second protrusion **102** and the second core **14**. A magnetic structure **16** is disposed between the second protrusion **102** and the second core **14**, and the magnetic structure **16** is symmetric with respect to the central line **CL** of the second protrusion **102**, as illustrated in FIG. 3 and FIG. 4A.

As the second protrusion **102** is located in the middle portion of the first core **10** and the magnetic structure **16** is disposed between the second protrusion **102** and the second core **14**, the magnetic structure **16** is located in the middle portion of the variable coupled inductor **1** after the variable coupled inductor **1** is fabricated. Furthermore, two ends of the magnetic structure **16** are respectively in full contact with the first core **10** and the second core **14**. In this embodiment, magnetic structure **16** is, but not limit to, in a long-strip shape. In this embodiment, the material of the first core **10**, the second core **14** and the magnetic structure **16** can be iron powder, ferrite, permanent magnet or other magnetic material. Because the first core **10** and the magnetic structure **16** are integrally formed, the material of the first core **10** is the same as that of the magnetic structure **16**. In another embodiment, the magnetic structure **16** and the second core **14** are also formed integrally, in such case, the material of the second core **14** is the same as that of the magnetic structure **16**. In another embodiment, the magnetic structure **16** can be also an independent device, in such case, the material of the magnetic structure **16** and the material of the first core **10**, or the second core **14**, can be the same or different. It should be noted that if the magnetic structure **16** is not in full contact with the first core **10** and the second core **14** due to manufacturing tolerance, magnetic glue can be filled in the gap (e.g., insulating resin and magnetic adhesive made of magnetic powder).

In this embodiment, the vertical distance **D1** of the first gap **G1** is smaller than the vertical distance **D2** of the second gap **G2**. The first gap **G1** can be an air gap, a magnetic gap and a non-magnetic gap, and the second gap **G2** can be also an air gap, a magnetic gap and a non-magnetic gap. The first gap **G1** and the second gap **G2** can be designed according to the practical application. It should be noted that the air gap is a gap filled with air for isolating and it does not contain other material; because air has a larger magnetic reluctance, it can increase degree of saturation of the inductor. The magnetic gap is formed by filling the magnetic material in the gap to reduce the magnetic reluctance and to further increase the inductance; as shown in FIG. 4B, non-magnetic gap is formed by filling the non-magnetic material **G1-M**, except the air, in the gap to enhance the function that the air gap can not achieve, such as by filling a bonding glue to combine different magnetic materials. Preferably, the first gap **G1** can be a non-magnetic gap, and the second gap **G2** can be an air gap or a non-magnetic gap.

In this embodiment, the variable coupled inductor **1** has a total high **H** after the variable coupled inductor **1** is fabricated; the vertical distance **D1** of the first gap **G1** can be in a range between 0.0073H and 0.0492H and the vertical distance **D2** of the second gap **G2** can be in a range between 0.0196H and 0.1720H. Furthermore, as illustrated in FIG. 4A, each of the first gap **G1** and the second gap **G2** lies within a height covered by the vertical distance **D3** between the bottom surface of the conducting-wire groove **104** and the second core **14**. In other words, when looking at the side

view shown in FIG. 4A, each top point of the first gap **G1** and the second gap **G2** is not higher than the top point of vertical distance **D3** between the bottom surface of the conducting-wire groove **104** and the second core **14**; and each bottom point of the first gap **G1** and the second gap **G2** is not lower than the bottom point of vertical distance **D3** between the bottom surface of the conducting-wire groove **104** and the second core **14**. In practical applications, the first gap **G1** generates a major inductance and the second gap **G2** generates a leakage inductance.

In this embodiment, the magnetic structure **16** has a first magnetic permeability  $\mu_1$ , the first gap **G1** has a second magnetic permeability  $\mu_2$ , and the second gap **G2** has a third magnetic permeability  $\mu_3$ , wherein the relationship between the first magnetic permeability  $\mu_1$ , the second magnetic permeability  $\mu_2$  and the third magnetic permeability  $\mu_3$  is  $\mu_1 > \mu_2 \geq \mu_3$ . In general, magnetic permeability is inversely proportional to the magnetic reluctance (i.e. the greater the magnetic permeability, the smaller the magnetic reluctance). The first magnetic permeability  $\mu_1$  of the magnetic structure **16** is larger than each of the second magnetic permeability  $\mu_2$  of the first gap **G1** and the third magnetic permeability  $\mu_3$  of the second gap **G2**, wherein the first gap **G1** and the second gap **G2** are located in two sides of the magnetic structure **16**, respectively. In other words, the magnetic reluctance of the magnetic structure **16** is smaller than that of the first gap **G1**; and the magnetic reluctance of the magnetic structure **16** is smaller than that of the second gap **G2**.

For example, the magnetic structure **16** can be manufactured by LTCC (low temperature co-fired ceramic, LTCC) printing; in such case, the first magnetic permeability  $\mu_1$  of the magnetic structure **16** is about between 50 and 200, and each of the second magnetic permeability  $\mu_2$  of the first gap **G1** and the third magnetic permeability  $\mu_3$  of the second gap **G2** is about 1. Because the first magnetic permeability  $\mu_1$  of the magnetic structure **16** is larger than each of the second magnetic permeability  $\mu_2$  of the first gap **G1** and the third magnetic permeability  $\mu_3$  of the second gap **G2**, the initial flux will passes through the magnetic structure **16** when a current passes through variable coupled inductor **1**. It should be noted that the first magnetic permeability  $\mu_1$  of the magnetic structure **16** is larger than each of the second magnetic permeability  $\mu_2$  of the first gap **G1** and the third magnetic permeability  $\mu_3$  of the second gap **G2** to achieve the effect of the variable inductance coupling regardless of the material of the first core **10** and the second core **14** (i.e. regardless of the magnetic permeability of the first core **10** and the second core **14**).

Furthermore, the first core **10** has a fourth magnetic permeability  $\mu_4$ , and the second core **14** has a fifth magnetic permeability  $\mu_5$ . For example, in another embodiment, when the magnetic structure **16**, the first core **10** and the second core **14** are all made of ferrite material, the first magnetic permeability  $\mu_1$ , the fourth magnetic permeability  $\mu_4$  and the fifth magnetic permeability  $\mu_5$  are the same. When the material of the magnetic structure **16** is ferrite material, the initial-inductance characteristic of the variable coupled inductor **1** can be enhanced and the efficiency of the variable coupled inductor **1** in a light-load situation can be improved as well. It should be noted that the relationship between the first magnetic permeability  $\mu_1$ , the second magnetic permeability  $\mu_2$ , the third magnetic permeability  $\mu_3$ , the fourth magnetic permeability  $\mu_4$  and the fifth magnetic permeability  $\mu_5$  is:  $\mu_1 \geq \mu_4 > \mu_2 \geq \mu_3$  and  $\mu_1 \geq \mu_5 > \mu_2 \geq \mu_3$ , regardless of the material of the magnetic structure **16**, the first core **10** and the second core **14**.

## 5

In summary, the present invention proposes that the magnetic structure **16** having a high magnetic permeability (i.e. the first magnetic permeability  $\mu_1$  described above) is disposed between the second projection **102** in the middle of the first core **10** and the second core **14**, and the magnetic structure **16** is symmetric with respect to the central line **CL** of the second protrusion **102**. Therefore, by using the magnetic structure **16**, the initial-inductance of the variable coupled inductor **1** can be enhanced and efficiency can be improved in a light-load situation.

Please refer to FIG. 5 and Table 1. FIG. 5 illustrates the relationship between the inductances and the currents measured in the variable coupled inductor **1** in FIG. 1, and table 1 lists the inductances and the currents in different measurements. As illustrated in FIG. 5, point A is a conversion point between light-load and heavy-lead situations (In this embodiment, the current at point A is, but not limited to, 10 A.) and the current at the point B is the maximum current to be expected to achieve (In this embodiment, the current at point B is, but not limited to, 50 A.). Herein, Light-load is called when the current is below the point A. From FIG. 5 and Table 1, the inductance of the variable coupled inductor **1** in a light-load situation is apparently enhanced, so that the variable coupled inductor **1** of the present invention can effectively improve light-load efficiency. It should be noted that, in this embodiment, the total height **H** of the variable coupled inductor **1** is about 4.07 mm, the vertical distance **D1** of the first gap **G1** is between 0.03 mm and 0.2 mm, and the vertical distance **D2** of the second gap **G2** is between 0.08 mm and 0.7 mm.

TABLE 1

| current (A) | inductance (nH) |
|-------------|-----------------|
| 0           | 599.6           |
| 5           | 269.8           |
| 10          | 159.35          |
| 11          | 154.38          |
| 12          | 150.52          |
| 13          | 147.55          |
| 14          | 145.29          |
| 15          | 143.61          |
| 20          | 138.05          |
| 25          | 134.3           |
| 30          | 131.45          |
| 35          | 129.3           |
| 40          | 127.4           |
| 45          | 125.5           |
| 50          | 123.6           |
| 55          | 121.7           |
| 60          | 119.8           |

In this embodiment, the magnetic structure **16** has a first surface area **A1**, and the second protrusion **102** has a second surface area **A2**. As illustrated in FIG. 3, the length of the magnetic structure **16** and the length of the second protrusion **102** are both **X**; the width of the magnetic structure **16** is **Y1**, and the width of the second protrusion **102** is **Y2**; the first surface area **A1** of the magnetic structure **16** is **X\*Y1**; the second surface area **A2** of the second protrusion **102** is **X\*Y2**. If the current at point A is defined as a first current **I1**, and the current at point B is defined as a second current **I2**, the relationship between the first current **I1**, the second current **I2**, the first surface area **A1** and the second surface area **A2** can be represented as  $1.21 (I1/I2) \geq A1/A2 \geq 0.81 (I1/I2)$ . Furthermore, a first inductance **L1** can be measured at the first current **I1**, and a second inductance **L2** can be measured at the second current **I2**; the relationship between the first inductance **L1** and the second inductance **L2** can be represented as  $0.8L1 \geq L2 \geq 0.7L1$ . In other words, the present invention proposes that the first inductance **L1** at the first current **I1** (i.e. the current at the conversion point between light-load and heavy-lead described above) and the second inductance **L2** at the second current **I2** (i.e. the maximum current to be expected to achieve) can be adjusted by adjusting the first surface area **A1** and the second surface **A2**.

## 6

It should be noted that the first current **I1** can be defined as follows. A third inductance **L3** is measured when the first current **I1** plus 1 amp is applied and  $5.5 \text{ nH} \geq L1 - L3 \geq 4.5 \text{ nH}$ . For example, the first current **I1** of this embodiment is 10 A, and the corresponding first inductance **L1** is 159.35 nH; the first current **I1** plus 1 equals 11 A, and the corresponding third inductance **L3** is 154.38 nH, wherein  $L1 - L3 = 4.97 \text{ nH}$  is obtained and  $5.5 \text{ nH} \geq 4.97 \text{ nH} \geq 4.5 \text{ nH}$  is satisfied. As defined above, when the current passes through the variable coupled inductor **1** in accordance with present invention, the corresponding current (i.e. the first current **I1** described above) at point A in FIG. 4A can be derived by measuring the inductance.

Please refer to FIG. 6. FIG. 6 is a three dimensional view of a first core **10** and a magnetic structure **16'** according to another embodiment of the present invention. The main difference between the magnetic structure **16** described above and the magnetic structure **16'** is that the length **X3** of the magnetic structure **16'** is smaller than the length **X** of the magnetic structure **16**, and the width **Y3** of the magnetic structure **16'** is larger than the width **Y1** of the magnetic structure **16**. In this embodiment, the surface area **X3\*Y3** of the magnetic structure **16'** is equal to the surface area **X\*Y1** of the magnetic structure **16**. Furthermore, a first portion **16a** of the magnetic structure **16'** is still symmetric to a second portion **16b** of the magnetic structure **16'** with respect to the central line **CL** of the second protrusion **102**. It should be noted that the magnetic structure **16'** and the first core **10** can be integrally formed or the magnetic structure **16'** and the second core **14** can be integrally formed. Alternatively, the magnetic structure **16'** can be an independent device.

Please refer to FIG. 7. FIG. 7 is a three dimensional view of a first core **10** and a magnetic structure **16''** according to another embodiment of the present invention. The main difference between the magnetic structure **16** described above and the magnetic structure **16''** is that the magnetic structure **16''** comprises two segments **160a**, **160b**, and the length and the width of each segment **160a**, **160b** are respectively **X4** and **Y4**. In this embodiment, the surface area  $(X4*Y4)*2$  of the magnetic structure **16''** is equal to the surface area **X\*Y1** of the magnetic structure **16**. Furthermore, the magnetic structure **16''** is still symmetric with respect to the central line **CL** of the second protrusion **102**, wherein a first portion **160a1** of the segment **160a** is symmetric to a second portion **160a2** of the segment **160a** with respect to the central line **CL** of the second protrusion **102**, and a first portion **160b1** of the segment **160b** is symmetric to a second portion **160b2** of the segment **160b** with respect to the central line **CL** of the second protrusion **102**. It should be noted that the magnetic structure **16''** and the first core **10** can be integrally formed or the magnetic structure **16''** and the second core **14** can be integrally formed. Alternatively, the magnetic structure **16''** can be an independent device.

Please refer to FIG. 8. FIG. 8 is a three dimensional view of a first core **10** and a magnetic structure **16'''** according to another embodiment of the present invention. The main difference between the magnetic structure **16** described above and the magnetic structure **16'''** is that the magnetic structure **16'''** comprises four segments **162a**, **162b**, **162c**,

**162d**, and the length and the width of each segment are **X5** and **Y5** respectively. In this embodiment, the surface area  $(X5*Y5)*4$  of the magnetic structure **16"** is equal to the surface area **X\*Y1** of the magnetic structure **16**. Furthermore, the magnetic structure **16"** is still symmetric with respect to the central line **CL** of the second protrusion **102**, wherein **162a** is symmetric to **162b** with respect to the central line **CL** of the second protrusion **102**, and **162c** is symmetric to **162d** with respect to the central line **CL** of the second protrusion **102**. That is, a first portion **162a**, **162c** of the four segments is symmetric to a second portion **162b**, **162d** of the four segments **162a**, **162b**, **162c**, **162d**. It should be noted that the magnetic structure **16"** and the first core **10** can be integrally formed or the magnetic structure **16"** and the second core **14** can be integrally formed. Alternatively, the magnetic structure **16"** can be an independent device.

In other words, the number of the segments and appearance of the magnetic structure can be designed in many ways as long as the same surface area is maintained. The magnetic structure is symmetric with respect to the central line **CL** of the second protrusion **102** regardless of the number of the segments and appearance of the magnetic structure

In conclusion, the present invention proposes that the magnetic structure is disposed between the second projection **102** in the middle of the first core **10** and the second core, and the magnetic structure is symmetric with respect to the central line **CL** of the second protrusion **102**. Therefore, the initial-inductance of the variable coupled inductor can be enhanced and light-load efficiency can be improved by means of the magnetic structure. Furthermore, the material of the variable coupled inductor of the present invention can be a ferrite material to achieve a high-saturation current, and copper sheet is used as an electrode to reduce the DC resistance, so efficiency is better in heavy-load. In other words, the variable coupled inductor of the present invention can improve efficiency in both light-load and heavy-load situations.

The above disclosure is related to the detailed technical contents and inventive features thereof. People skilled in this field may proceed with a variety of modifications and replacements based on the disclosures and suggestions of the invention as described without departing from the characteristics thereof. Nevertheless, although such modifications and replacements are not fully disclosed in the above descriptions, they have substantially been covered in the following claims as appended.

What is claimed is:

1. A variable coupled inductor, comprising:  
a first core having a top surface and a bottom surface, a first lateral surface and a second lateral surface opposite to the first lateral surface, wherein the first core comprises a first protrusion, a second protrusion, a third protrusion, a first conducting-wire groove and a second conducting-wire groove, each of which extending from the first lateral surface to the second lateral surface on the top surface, wherein the second protrusion is disposed between the first protrusion and the third protrusion, wherein the first conducting-wire groove is located between the first protrusion and the second protrusion, and the second conducting-wire groove is located between the second protrusion and the third protrusion;  
a first conducting wire disposed in the first conducting-wire groove and  
a second conducting wire disposed in the second conducting-wire groove;  
a second core disposed over the first core; and

a magnetic structure disposed between the second protrusion and the second core, wherein the magnetic structure comprises a first portion and a second portion, wherein the first portion and the second portion are symmetric to each other with respect to a central line of the second protrusion, wherein the central line extends from a first middle point of a first edge of the second protrusion on the first lateral surface to a second middle point of a second edge of the second protrusion on the second lateral surface, wherein side surfaces of the second protrusion located below said magnetic structure are not used for winding a conductive wire therearound, wherein a top surface of the second protrusion is respectively lower than a top surface of the first protrusion and a top surface of the third protrusion, and a top surface of said magnetic structure is respectively higher than said top surface of the first protrusion and said top surface of the third protrusion.

2. The variable coupled inductor according to claim 1, wherein the magnetic structure comprises at least two segments separated from each other, wherein the at least two segments has a first portion and a second portion that are symmetric with each other with respect to the central line of the second protrusion.

3. The variable coupled inductor according to claim 1, wherein a first gap is formed between the first protrusion and the second core, a second gap is formed between the second protrusion and the second core and a third gap is formed between the third protrusion and the second core, wherein the vertical distance of each of the first gap and the third gap is smaller than that of the second gap, wherein the variable coupled inductor has a height **H**, the vertical distance of each of the first gap and the third gap is between  $0.0073H$  and  $0.0492H$ , and the vertical distance of the second gap is between  $0.0196H$  and  $0.1720H$ .

4. The variable coupled inductor according to claim 3, wherein the magnetic structure has a first magnetic permeability  $\mu_1$ , each of the first gap and the third gap has a second magnetic permeability  $\mu_2$ , and the second gap has a third magnetic permeability  $\mu_3$ , wherein the relationship between the first magnetic permeability  $\mu_1$ , the second magnetic permeability  $\mu_2$  and the third magnetic permeability  $\mu_3$  is:  $\mu_1 > \mu_2 \geq \mu_3$ .

5. The variable coupled inductor according to claim 3, wherein the first core has a fourth magnetic permeability  $\mu_4$ , and the second core has a fifth magnetic permeability  $\mu_5$ , wherein the relationship between the first magnetic permeability  $\mu_1$ , the second magnetic permeability  $\mu_2$ , the third magnetic permeability  $\mu_3$ , the fourth magnetic permeability  $\mu_4$  and the fifth magnetic permeability  $\mu_5$  is:  $\mu_1 \geq \mu_4 > \mu_2 \geq \mu_3$  and  $\mu_1 \geq \mu_5 > \mu_2 \geq \mu_3$ .

6. The variable coupled inductor according to claim 3, wherein each of the first gap, the second gap and the third gap lies in a height covered by the vertical distance between the bottom surface of the first conducting-wire groove and the second core.

7. The variable coupled inductor according to claim 1, wherein a first gap is formed between the first protrusion and the second core, wherein the first gap is filled with a non-magnetic material.

8. The variable coupled inductor according to claim 1, wherein a first gap is formed between the first protrusion and the second core, and a second gap is formed between the second protrusion and the second core, wherein each of the first gap and the second gap is filled with a non-magnetic material.

9. The variable coupled inductor according to claim 1, wherein the magnetic structure and the second core are integrally formed.

10. The variable coupled inductor according to claim 1, wherein the magnetic structure and the second core are integrally formed, and the magnetic structure has a magnetic permeability  $\mu_1$  and the first core has a magnetic permeability  $\mu_4$ , wherein  $\mu_1 > \mu_4$ .

11. A variable coupled inductor, comprising:

a first core having a top surface and a bottom surface, a first lateral surface and a second lateral surface opposite to the first lateral surface, wherein the first core comprises a first protrusion, a second protrusion, a third protrusion, a first conducting-wire groove and a second conducting-wire groove, each of which extending from the first lateral surface to the second lateral surface on the top surface, wherein the second protrusion is disposed between the first protrusion and the third protrusion, wherein the first conducting-wire groove is located between the first protrusion and the second protrusion, and the second conducting-wire groove is located between the second protrusion and the third protrusion;

a first conducting wire disposed in the first conducting-wire groove and

a second conducting wire disposed in the second conducting-wire groove;

a second core disposed over the first core; and

a magnetic structure disposed between the second protrusion and the second core, wherein the magnetic structure comprises at least one segment, wherein the at least one segment has a first portion and a second portion that are symmetric with each other with respect to a central line of the second protrusion, wherein the central line extends from a first middle point of a first edge of the second protrusion on the first lateral surface to a second middle point of a second edge of the second protrusion on the second lateral surface, wherein side surfaces of the second protrusion located below said magnetic structure are not used for winding a conductive wire therearound, wherein a top surface of the second protrusion is respectively lower than a top surface of the first protrusion and a top surface of the third protrusion, and a top surface of said magnetic structure is respectively higher than said top surface of the first protrusion and said top surface of the third protrusion.

12. The variable coupled inductor according to claim 11, wherein a first gap is formed between the first protrusion and the second core, wherein the first gap is filled with a non-magnetic material.

13. The variable coupled inductor according to claim 11, wherein the magnetic structure has a magnetic permeability  $\mu_1$  and the first core has a magnetic permeability  $\mu_4$ , wherein  $\mu_1 > \mu_4$ .

14. The variable coupled inductor according to claim 11, wherein the magnetic structure and the second core are integrally formed.

15. The variable coupled inductor according to claim 11, wherein the magnetic structure and the second core are

integrally formed, and the magnetic structure has a magnetic permeability  $\mu_1$  and the first core has a magnetic permeability  $\mu_4$ , wherein  $\mu_1 > \mu_4$ .

16. A variable coupled inductor, comprising:

a first core having a top surface and a bottom surface, a first lateral surface and a second lateral surface opposite to the first lateral surface, wherein the first core comprises a first protrusion, a second protrusion, a third protrusion, a first conducting-wire groove and a second conducting-wire groove, each of which extending from the first lateral surface to the second lateral surface on the top surface, wherein the second protrusion is disposed between the first protrusion and the third protrusion, wherein the first conducting-wire groove is located between the first protrusion and the second protrusion, and the second conducting-wire groove is located between the second protrusion and the third protrusion;

a first conducting wire disposed in the first conducting-wire groove and

a second conducting wire disposed in the second conducting-wire groove, wherein the first conducting wire and the second conducting wire are extended to wrap around the first core at two opposite sides of the second protrusion of the first core via the bottom surface;

a second core disposed over the first core; and

a magnetic structure disposed between the second protrusion and the second core, wherein the magnetic structure comprises a first portion and a second portion that are symmetric with each other with respect to a central line of the second protrusion, wherein the central line extends from a first middle point of a first edge of the second protrusion on the first lateral surface to a second middle point of a second edge of the second protrusion on the second lateral surface, wherein the magnetic structure and the second core are integrally formed, wherein side surfaces of the second protrusion located below said magnetic structure are not used for winding a conductive wire therearound, wherein a top surface of the second protrusion is respectively lower than a top surface of the first protrusion and a top surface of the third protrusion, and a top surface of said magnetic structure is respectively higher than said top surface of the first protrusion and said top surface of the third protrusion.

17. The variable coupled inductor according to claim 16, wherein the magnetic structure has a magnetic permeability  $\mu_1$  and the first core has a magnetic permeability  $\mu_4$ , wherein  $\mu_1 > \mu_4$ .

18. The variable coupled inductor according to claim 16, wherein the magnetic structure and the second core are integrally formed, and the magnetic structure has a magnetic permeability  $\mu_1$  and the first core has a magnetic permeability  $\mu_4$ , wherein  $\mu_1 > \mu_4$ .